

## UNITED STATES PATENT OFFICE

2,584,280

METHOD OF PREPARING SUBSTANTIALLY  
IRON-FREE AMMONIUM SULFATE FROM  
SPENT PICKLE LIQUOR

Herman P. Meissner, Watertown, and Richard W. Hyde, Arlington, Mass., assignors, by mesne assignments, to Republic Steel Corporation, Cleveland, Ohio, a corporation of New Jersey

No Drawing. Application January 9, 1947,  
Serial No. 721,152

3 Claims. (Cl. 23—119)

1

The present invention relates generally to the art of synthesizing compounds of iron and of ammonia, and is particularly concerned with a novel method for preparing, from coke oven gas and spent pickle liquor, iron compounds substantially free from ammonium sulfate and high purity ammonium sulfate substantially uncontaminated by iron or iron compounds.

In the conventional practice for pickling iron and steel bars, sheets and other shapes, wherein a hot sulfuric acid bath is employed, the pickling bath is reused with addition of more acid as required, until it becomes unsatisfactory for further use because it is too saturated with salts or too heavily loaded with dirt and sediment. This spent liquor from continuous picklers typically contains 18 to 22% ferrous sulfate and 3 to 12% sulfuric acid, while that from batch picklers typically contains 20 to 30% ferrous sulfate plus 1 to 3% sulfuric acid, by processes now commonly used commercially. Also present in the liquor are traces of sulfates of other metals associated with the pickled iron or steel as alloying elements or impurities.

This spent pickling liquor must be disposed of. Many attempts have been made economically to recover the chemical values in pickle liquor. In the processes developed to date, costs of recovery have generally exceeded the value of the products recovered. The usual procedure has therefore involved disposal in the most inexpensive manner consistent with standards of health, sanitation, and stream pollution obtaining in that particular locality. As these standards become more rigid, the older practice of dumping into streams has in many instances been abolished, and some alternative procedure such as neutralizing with lime and dumping the resultant precipitate has been adopted. Practically all these procedures have the objective of getting rid of the pickle liquor as expeditiously as possible, rather than the conservation of any of its values. An economic process for accomplishing the latter objective has long been desired.

By virtue of the present invention, which involves not only the useful employment of spent pickle liquor but also beneficiation of coke oven gases, the foregoing demand is met and an economical process for simultaneously disposing of spent pickle liquor and converting its chemical values into useful form, is available. This invention has the added advantage that the method thereof is readily controllable to produce the desired results, coke oven gas employed is freed from undesirable prussic acid, hydrogen sulfide

2

and ammonia which are converted into valuable substances, and coke oven gas and spent pickle liquor of a wide variety of compositions may be treated with the same results in routine manner.

Briefly stated, the process of our present invention comprises the step of contacting a suitable ammonia-containing gas with a spent pickle liquor until the pH of the resulting solid-liquid mixture is between about 8.1 and about 8.5 and thereby precipitating substantially all the chemically combined iron present in said liquor.

In carrying out this invention, coke oven gas or other similarly effective ammonia-containing gas, is suitably contacted with the waste pickle liquor. This might be done countercurrently, for example, in absorption towers packed with wide-spaced wooden grids to minimize plugging hazards due to precipitate formation. Operations should be so adjusted that the reacted pickle liquor, also called the black slurry product because of its typical color and its solid-liquid constitution, leaves the system with a minimum dissolved iron content, which corresponds to a pH in the range between about 8.1 and about 8.5, and preferably at a pH of about 8.3. Only under these conditions can a black slurry product be made from which the separation of the precipitated iron salts by filtration, centrifuging or settling can be readily attained while simultaneously leaving behind a solution containing ammonium sulfate relatively uncontaminated with dissolved iron, sulfide or cyanide compounds. Moreover, if sufficient gas-liquor contact is provided, this necessary control of the exit liquor can be accomplished while attaining extensive removal of ammonia from the coke oven gas, together with most of the cyanide and at least part of the H<sub>2</sub>S.

The precipitated solids and clear liquor from the black liquor separation must be handled separately. The precipitated solids are washed to recover entrained ammonium sulfate solution, and can then be sintered preparatory to being charged to a blast furnace, or processed for recovery of cyanide or other values, or used in the removal of further amounts of H<sub>2</sub>S from the deammoniated coke oven gas, otherwise disposed of. On the other hand, the clear liquor from the black slurry separation can, if desired, be exposed to the air for a while to oxidize the small amount of dissolved iron present to the ferric state, whereupon the ferric hydroxide formed can be removed by filtration or otherwise treated. Another optional step would involve adding sulfuric acid to convert the small amount of dissolved free ammonia present to sulfate, since

this ammonia would otherwise be lost in the subsequent evaporation. This final evaporation step can be carried out in any suitable equipment, and the ammonium sulfate crystal product recovered. The bottoms liquor from the evaporators can be recycled to the absorption towers along with the fresh pickle liquor feed.

The importance of correct control of the black slurry composition is illustrated by the following experiment on coke oven gas, which typically analyzes 1% NH<sub>3</sub>, 0.7% H<sub>2</sub>S, 0.1% HCN, 2.3% CO<sub>2</sub> and the balance chiefly CO, H<sub>2</sub>, CH<sub>4</sub>, and illuminants. Upon bubbling such a gas through pickle liquor, located for example in a laboratory absorption bottle, at least three major stages in the absorption can be detected. During the first stage, no precipitate forms due to the presence of free acid, and the ratio of dissolved iron to sulfate in solution remains constant. The second stage shows the formation of blue-black precipitate of iron compounds, and so is characterized by a falling ratio of dissolved iron to sulfate in solution as more and more gas passes through the solution. The critical or optimum point is finally reached, at which the amount of dissolved iron, and similarly the ratio of dissolved iron to sulfate, is a minimum. In the third stage, the amount of iron in solution increases due to a redissolving of the precipitated iron compounds, and so this third stage is characterized by an increasing ratio of dissolved iron to sulfate in solution.

The reactions during these three stages are quite complex. In stage one, probably little CO<sub>2</sub>, HCN or H<sub>2</sub>S dissolve, since these gases are relatively insoluble in acid solutions, and since they cannot form precipitates with iron in the presence of acid. The chief reaction occurring here, therefore, is probably the neutralization of the free acid in the pickle liquor with the absorbed ammonia. In the second stage, iron precipitates due to the reaction:



Iron precipitation due to the formation of sulfides, carbonates, and cyanides also occurs, as is shown by the following typical analysis of an (unwashed) precipitate removed from a solution at the critical point between stages two and three of the absorption:

|                                 | Per cent |
|---------------------------------|----------|
| Loss at 105° C-----             | 72.98    |
| Sulfide sulfur -----            | 9.65     |
| Sulfate sulfur -----            | 2.16     |
| Total nitrogen (Kjeldahl) ----- | 3.36     |
| Total ammonia -----             | 2.88     |
| Free ammonia -----              | 0.34     |
| Cyanide (by difference) -----   | 1.83     |
| Carbon dioxide-----             | 0.05     |

The iron sulfides, cyanides and carbonates are all relatively insoluble at this critical point at the end of stage two, for the liquid phase now shows a minimum amount of these contaminants in solution, and therefore chiefly contains dissolved ammonium sulfate and a little free ammonia. During stage three, however, the increasing alkalinity of the solution due to the absorption of ammonia results in further absorption of hydrogen sulfide and cyanide. Simultaneously, the precipitated iron compounds still present begin to go back into solution, probably due to the formation of soluble iron salts such as iron thiocyanide, ammonium ferrocyanide, etc.

The important finding here is the necessity of operating so that the pickle liquor is brought to the critical point at the end of stage two. If an excess of gas is treated, so that stage three is entered upon, then the solution is contaminated with sulfides, cyanides, and redissolved iron compounds. If an insufficiency of gas is passed through the pickle liquor so that the critical point at the end of stage two is not reached, then the iron in the pickle liquor is not entirely precipitated. In either case, the solution of ammonium sulfate is contaminated with dissolved iron and other compounds, which makes the recovery of pure ammonium sulfate crystals by evaporation very difficult.

The iron precipitate formed is extremely fine, and of a somewhat slimy, gelatinous nature. It appears to improve somewhat in filterability with increasing pH. At the critical pH of 8.3, this precipitate has been found to separate readily from the liquid phase in a high speed centrifuge. Filtration is somewhat more difficult, but can be carried out successfully, especially if a little filter-aid is used.

The control of absorption operations, so that the black slurry produced will be at the desired critical point at the end of stage two, may be accomplished in several ways. A most convenient procedure was found to involve following the course of the reaction by determining the hydrogen ion concentration of the pickle liquor during absorption with a standard pH meter. Fresh pickle liquor has a variable hydrogen ion concentration depending on its composition, but typically might have a pH about 2.0. As absorption proceeds, the pH increases until it is about 8.3 which is the critical point. If now the absorption is allowed to proceed further, the final pH reached is perhaps 10. It was found that the pH range between about 8.1 and about 8.5 could be used as an accurate indication that the critical point had been reached, regardless of the ratio of ferrous sulfate to free acid in the original pickle liquor or the concentration of these components in the liquor. This critical pH value also varied little with such typical changes in the analysis of the coke oven gases as might be encountered in industrial coke plant operation. Temperature of absorption likewise appeared to have little effect on the critical pH value.

Control of absorption might also be achieved by any means for determining the ratio of iron to sulfate in solution in the liquid phase of the black slurry, as for example by chemical analysis. Adequate control could also be accomplished by operating to obtain a minimum concentration of dissolved iron, which might be determined by color or other suitable procedure.

The operation of this process on a larger scale might advantageously involve a continuous countercurrent contacting of the pickle liquor and the coke oven gas. This contacting might be accomplished in absorption towers packed with wooden slats, stone, Raschig rings, or similar materials, or it might be carried out in a conventional spray or bubble cap tower. The countercurrent operation of a series of stage contacts, such as the "saturators" now installed extensively in coke plants for ammonia recovery, would also be suitable. In other words, any orthodox gas-liquor contacting device which will not plug up with precipitate, can be used.

In the event that towers are used, the pickle liquor would ordinarily flow down countercurrent to the ascending gas stream. The relative

rates of feed of gas and liquor to the towers would be so adjusted that the black slurry product would be at the critical point between stages two and three of the reaction described above, or in other words, contain a minimum iron content and so have a pH between about 8.1 and about 8.5. If in actual operation, for example, a tower system was found to produce a product of too low pH (under-reacted), then it is merely necessary to decrease the rate of liquor flow relative to the gas flow to improve the pH of the product to the proper value. If, on the contrary, too high a pH value is evident, then an increase of liquor flow relative to the gas will correct this difficulty.

It is evident that, if sufficient gas-liquid contact is supplied, an extensive recovery of ammonia from the gas becomes possible even while producing a black slurry product of the desired pH. It was, for example, found possible to recover 97% of the NH<sub>3</sub> in a synthetic coke oven gas when operating with a two-stage gas-liquor contact, with countercurrent flow. Simultaneously, the hydrogen cyanide present is also extensively removed from the gas by this scrubbing operation (80 to 90%) along with a part of the hydrogen sulfide present (30-40%). Such removal is desirable, since the toxicity of HCN makes it a hazardous component in any fuel, especially for domestic use, while H<sub>2</sub>S has further disadvantages as a fuel gas component if used for steel making and the like.

The fact that the critical pH is largely independent of the concentration and the ratio of acid to ferrous sulfate in the pickle liquor, as discussed above, is advantageous from an operating point of view in two ways. First, the waste pickle strength and proportions as produced in a steel plant may vary considerably depending upon a number of factors. Second, it is rare that a steel plant produces pickle liquor and coke oven gases in correct proportions for absorption, and any deficit in pickle liquor is most easily made up by sulfuric acid additions. As proposed here, operation with pH control, or control by critical concentration of iron in solution, is feasible even though the pickle liquor undergoes large variations in concentration and analysis.

The iron precipitate can be separated from the black liquor slurry by centrifuging or otherwise. This precipitate must then be washed to recover the entrained ammonium sulfate, and this washing can be done on the centrifuge or filter used, or by repulping, or similar orthodox procedures. The wash water can then be evaporated to recover ammonium sulfate. The precipitated iron salts, after washing, typically analyze on a wet basis about 75% water, 7% sulfide sulfur, somewhat under 7% CN, and the remainder chiefly iron. This analysis will of course vary somewhat, depending upon the composition of the liquor and gas used. As already indicated, these solids can now be put to one or another of various uses, e. g. dried and sintered for blast furnace use, or treated to recover cyanide or other values, etc.

The liquor left after separating the iron precipitate from the black slurry contains a small amount of ferrous iron in solution. The evaporation of this liquor without further treatment yields ammonium sulfate of good purity. In a run using typical gas and pickle liquor, it was found that ammonium sulfate containing only 0.09% iron by weight could be made in this

fashion. If desired, however, this purity can be further improved e. g. to 0.004% by weight by first oxidizing the liquor by exposure to air or oxygen. The ferric hydroxide which forms can be separated by filtration, settling, or other methods. The suspension can also be sent direct to the evaporators without previous solids separation, since it appears that the ammonium sulfate crystals formed here by evaporation are relatively uncontaminated by the ferric hydroxide floc, providing too great a percentage of the water present is not evaporated off. The bottoms liquor containing the ferric hydroxide floc is then recycled to the absorption towers along with the fresh pickle liquor feed.

The desirability of neutralizing the free ammonia in the liquor before sending it to the evaporators has been mentioned. If this is not done, this free ammonia will be lost, or must somehow be recovered from the vapors in the evaporators.

Having thus described the present invention so that others may be able to understand and practice the same, we state that what we desire to secure by Letters Patent is defined in what is claimed.

What is claimed is:

1. The method of precipitating as ferrous compounds substantially all the chemically combined iron of a spent pickle liquor which comprises the steps of contacting said liquor with a crude coke oven gas containing ammonia to elevate and maintain the pH of said liquor between about 8.1 and about 8.5 and thereby converting the said liquor into a black slurry containing precipitated ferrous compounds, and separating the solid phase from the liquid phase which consists essentially of ammonium sulfate and contains substantially no dissolved iron.

2. The method of precipitating as ferrous compounds substantially all the chemically combined iron of a spent pickle liquor which comprises the steps of continuously bringing a crude coke oven gas containing ammonia into contact with said liquor to elevate and maintain the pH of said liquor between about 8.1 and about 8.5 and thereby converting said liquor into a black slurry containing precipitated ferrous iron compounds, and separating the solid phase from the liquid phase which consists essentially of ammonium sulfate and contains substantially no dissolved iron.

3. The method of precipitating as ferrous compounds substantially all the chemically combined iron of a spent pickle liquor which comprises the steps of continuously flowing said liquor in countercurrent contact with a stream of a crude coke oven gas containing ammonia to elevate and maintain the pH of said liquor between about 8.1 and about 8.5 and thereby converting the said liquor into a black slurry containing precipitated ferrous iron compounds, and separating the solid phase from the liquid phase which consists essentially of ammonium sulfate and contains substantially no dissolved iron.

4. The method of producing from a spent pickle liquor ferrous iron compounds substantially uncontaminated by sulfates which comprises the steps of contacting said liquor with a crude coke oven gas containing ammonia to elevate and maintain the pH of said liquor between about 8.1 and about 8.5 and thereby converting the said liquor into a black slurry containing precipitated ferrous iron compounds, separating the solid phase from the liquid phase which consists essentially of ammonium sulfate and contains substantially no dissolved iron, and washing the solid

phase material with water substantially free of sulfate.

5. The method of preparing substantially iron-free ammonium sulfate from a spent pickle liquor which comprises the steps of contacting said liquor with a crude coke oven gas containing ammonia to elevate and maintain the pH of said liquor between about 8.1 and 8.5 and thereby converting the said liquor into a black slurry containing precipitated ferrous iron compounds, separating the solid phase from the liquid phase which consists essentially of ammonium sulfate and contains substantially no dissolved iron, contacting said liquid phase with an oxidizing gas and oxidizing any residual dissolved iron, and separating the ammonium sulfate from the resulting precipitate of oxidized iron.

6. The method of preparing substantially iron-free ammonium sulfate from a spent pickle liquor which comprises the steps of contacting said liquor with a crude coke oven gas containing ammonia to elevate and maintain the pH of said liquor between about 8.1 and about 8.5 and thereby converting the said liquor into a black slurry containing precipitated ferrous iron compounds, separating the solid phase from the liquid phase which consists essentially of ammonium sulfate and contains substantially no dissolved iron, contacting said liquid phase with an oxidizing gas and oxidizing any residual dissolved iron, partially evaporating the liquid phase and crystallizing the ammonium sulfate therein, and removing the ammonium sulfate crystals from the mother liquor containing oxidized iron in solid form and separating the ammonium sulfate from the resulting precipitate of oxidized iron.

7. The method of preparing substantially iron-free, crystalline ammonium sulfate of high purity from a spent pickle liquor which comprises the steps of contacting said liquor with a crude coke oven gas containing ammonia to elevate and maintain the pH of said liquor between about 8.1 and about 8.5 and thereby converting the said

liquor into a black slurry containing precipitated ferrous iron compounds, separating the solid phase which consists essentially of ammonium sulfate and contains substantially no dissolved iron, contacting said liquid phase with air and thereby oxidizing any residual dissolved iron, separating iron thus oxidized and precipitated from the liquid phase, and crystallizing the ammonium sulfate from the liquid phase by evapo-

10 rating a portion of said liquid phase.

8. The method of continuously preparing from a spent pickle liquor substantially iron-free, crystalline, high purity ammonium sulfate which comprises the steps of continuously flowing said liquor in countercurrent contact with a crude coke oven gas containing ammonia to elevate and maintain the pH of said liquor between about 8.1 and about 8.5 and thereby converting the said liquor into a black slurry containing precipitated ferrous iron compounds, continuously withdrawing portions of the liquor from contact with the gas as the pH of these portions reaches a predetermined value between about 8.1 and about 8.5, separating the solid phase of these said portions from the liquid phase thereof which consists essentially of ammonium sulfate and contains substantially no dissolved iron, and continuously evaporating said liquid phase of these portions and crystallizing ammonium sulfate therefrom.

30 HERMAN P. MEISSNER.  
RICHARD W. HYDE.

#### REFERENCES CITED

The following references are of record in the file of this patent:

#### UNITED STATES PATENTS

| Number       | Name    | Date           |
|--------------|---------|----------------|
| 961,763      | Falding | June 21, 1910  |
| 40 1,983,320 | Sperr   | Dec. 4, 1934   |
| 2,419,240    | Wilson  | Apr. 22, 1947  |
| 2,427,555    | Elzi    | Sept. 16, 1947 |
| 2,443,765    | Francis | June 22, 1948  |